

## UNITED STATES PATENT OFFICE

2,357,876

DEEP DRAWING STEELS AND METHOD OF  
MAKING THE SAME

Walter Crafts and Cecil G. Chadwick, Niagara Falls, N. Y., assignors to Electro Metallurgical Company, a corporation of West Virginia

No Drawing. Application December 1, 1942,  
Serial No. 467,553

6 Claims. (Cl. 75—123)

The invention relates to deep drawing steels, to deep drawn articles made therefrom and to a method for preparing deep drawn steel.

Deep drawing steels of the low carbon, aluminum-killed type are currently employed in large quantity by industry. Silicon-killed steels are, in general, less satisfactory due to the hardening effect of the silicon addition.

It is the primary object of the present invention to provide a silicon-killed steel having good deep drawing properties. Another object is to provide deep drawn articles having smooth surface characteristics. A further object is to provide a silicon-killed deep drawing steel of uniform grain size, the properties of which are comparable to plain, aluminum-killed deep drawing steels. A still further object is to provide a method of preparing deep drawn steel of silicon-killed steel.

These and other objects are achieved by the invention which is based on the discovery that boron exerts a softening effect in low-carbon deep drawing steels and that this effect may be utilized to compensate for the hardening effect of silicon. By substituting silicon for the normal or part of the normal aluminum addition in low-carbon deep drawing steels and additionally treating such steels with boron, properties comparable to those of aluminum-killed deep drawing steels may be obtained.

The invention in its broader aspect comprises deep drawing steels or articles made therefrom containing between 0.01% and 0.10% carbon, 0.10% to 1% manganese, 0.05% to 0.50% silicon, 0.0005% to .05% boron, remainder iron and incidental impurities such as normally occur in the manufacture of low carbon steels of good quality. In a preferred embodiment of the invention, the upper limit of manganese below 0.50%, the upper limit of silicon below 0.30% and the boron between 0.001% and 0.02%. Although steels containing silicon in rather large amounts may be benefited by treatment with boron, it nevertheless appears advisable to limit the silicon addition to the lowest amount consistent with good deoxidation practice.

In accordance with the present invention, deep drawn articles may be made by preparing a low carbon steel melt containing carbon in an amount less than 0.10%, treating the melt with silicon in any desired form, as for example, ferrosilicon, in an amount sufficient to deoxidize the melt but insufficient to leave a residual silicon content greater than 0.50%, preferably no greater than 0.30%, adding boron in an amount

sufficient to counteract the hardening effect of the silicon addition, the boron addition being between 0.0005% and 0.05%, preferably between 0.001% and 0.02%, casting the resulting steel melt and rolling the same to sheet and thereafter subjecting to a pressing operation to form a deep drawn article.

The boron addition may be made in almost any convenient form. For example, it may be added as an oxide or a salt, such as borax; as a boride or other compound, such as boron carbide; as a metallic alloy, such as manganese-boron or calcium-boron; or it may be added in combination with silicon in the form of a ferrosilicon-boron alloy or in combination with manganese and silicon in the form of an iron-manganese-silicon-boron. Although the invention is not limited to the use of any specific agent for adding boron, and the types of agents just mentioned

are merely suggestive of the wide range of possible means by which the boron addition may be made to the steel, nevertheless under some conditions particularly favorable results are obtainable by the use of an agent consisting essentially of silicon, manganese, boron and iron in appropriate relative proportions. Preferred proportions comprise 20% to 60% silicon, 60% to 20% manganese, 1% to 15% boron, remainder iron and other incidental impurities.

Due to the existence of many external factors which enter into deep drawing operations, there is no single standard test which can be directly interpreted in terms of commercial deep drawing properties. Among the variables encountered in the deep drawing of steel are the type of lubricant employed, the die construction, the rate of draw, and the surface finish required on the final deep drawn article. There are, however, certain physical properties, determinable by simple testing, which are accepted as indicia of the relative deep drawing characteristics of steels. In general, these properties are low yield point, moderately low tensile strength and hardness, good elongation as measured by percentage elongation in tensile test, depth of cup in cupping test, and substantial freedom from aging effects.

The excellent properties obtained by utilizing silicon as a deoxidizing agent and additionally treating the silicon-killed steels with boron is shown in Tables A and B in which Table A sets forth the compositions of the steels and Table B the physical properties. The steels of the series were all deoxidized in the furnace, cross-rolled to form sheets 0.05 inch in thickness, sandblast-

ed and pack annealed. After annealing, the sheets were pickled and cold-rolled to 0.04 inch in thickness. The cold-rolled sheets were then annealed at the temperatures indicated in Table B, pickled, and finally given a cold roll pinch pass equivalent to two per cent reduction. One set of specimens was tested after the foregoing treatment. A corresponding set of annealed specimens was tested after the foregoing treatment plus an accelerated aging treatment that comprised heating the specimens at 200° C. for 24 hours in an air atmosphere. A visible oxide formed on the specimens due to the aging treatment, which oxide was not removed prior to testing the specimens.

In Table B, "Y. P." means yield point in pounds per square inch; "T. S." means tensile strength in pounds per square inch; "% El" means percentage elongation in a gauge length of two inches; "Hardness RB" means the hardness value on the Rockwell "B" scale; "Erichsen" means the greatest depth of indentation measured in millimeters made in the Erichsen cupping test before incipient cracking of the sheet; and "A. S. T. M. grain size" means the actual grain size as measured according to the American Society for Testing Materials grain size index.

TABLE A  
Composition of steels by chemical analysis  
(remainder substantially iron)

| Steel No. | Percent C | Percent Mn <sup>1</sup> | Percent Si | Percent Al <sup>2</sup> | Percent B <sup>2</sup> |
|-----------|-----------|-------------------------|------------|-------------------------|------------------------|
| 1-----    | 0.04      | 0.30                    | 0.03       | 0.20                    | -----                  |
| 2-----    | 0.07      | 0.30                    | 0.16       | -----                   | -----                  |
| 3-----    | 0.04      | 0.30                    | 0.05       | -----                   | 0.01                   |
| 4-----    | 0.07      | 0.30                    | 0.18       | -----                   | 0.01                   |
| 5-----    | 0.05      | 0.30                    | 0.21       | -----                   | 0.01                   |

<sup>1</sup> Nominal analysis.

<sup>2</sup> Added amount.

TABLE B  
Physical properties

| Steel No. | Heat treatment after cold rolling | Y. P.  | T. S.  | Per cent El | Hardness RB | Erichsen | A. S. T. M. grain size |
|-----------|-----------------------------------|--------|--------|-------------|-------------|----------|------------------------|
| 1-----    | Annealed (1)-----                 | 23,850 | 44,750 | 38          | 39          | 11.7     | 5                      |
| 1-----    | Annealed (1) and aged-----        | 33,750 | 45,650 | 34          | 47          | 11.4     | -----                  |
| 2-----    | Annealed (1)-----                 | 32,550 | 53,450 | 29          | 53          | 11.1     | 5                      |
| 2-----    | Annealed (1) and aged-----        | 37,500 | 51,700 | 28          | 59          | 10.8     | -----                  |
| 3-----    | Annealed (2)-----                 | 23,750 | 42,800 | 35          | 33          | 11.8     | 5                      |
| 3-----    | Annealed (2) and aged-----        | 32,200 | 42,750 | 40          | 40          | 11.7     | -----                  |
| 4-----    | Annealed (1)-----                 | 27,600 | 48,050 | 36          | 44          | 11.5     | 5                      |
| 4-----    | Annealed (1) and aged-----        | 35,650 | 48,950 | 33          | 50          | 11.0     | -----                  |
| 5-----    | Annealed (2)-----                 | 27,850 | 47,950 | 36          | 34          | 11.4     | 5-6                    |
| 5-----    | Annealed (2) and aged-----        | 36,050 | 49,000 | 33          | 43          | 11.4     | -----                  |

Annealed (1)=925° C.—furnace cool to 710° C., 8 hours—furnace cool.

Annealed (2)=925° C.—air cool, 710° C., 8 hours—furnace cool.

Aged=200° C.—24 hours—air cool.

In the tables, Steel No. 1 is a low carbon aluminum-killed steel of typical physical properties, such as currently employed in industry for deep drawing purposes. Steel No. 2 is a plain low carbon steel in which silicon was employed as the deoxidizing agent for killing the steel. It will be noted that the yield point of the silicon-killed steel (No. 2) is considerably higher than that of the aluminum-killed steel (No. 1) and further that the silicon-killed steel is harder, has less elongation, and less cupping depth than the aluminum-killed steel. This condition exists in both the annealed and in the annealed and aged state. Steels Nos. 3, 4 and 5 are silicon-killed steels of increasing silicon content which have been treat-

ed with a boron addition according to the invention. The softening effect of the boron addition to the silicon-killed steels may be seen by a comparison of Steels Nos. 3, 4 and 5 with the plain silicon-killed Steel No. 2. This comparison shows that the boron additions have effected a lowering of the yield point, tensile strength and hardness and have increased the ductility as measured by the percentage elongation and Erichsen values while maintaining a uniform grain size.

As indicated by these data, silicon when added alone for purposes of deoxidation, hardens and strengthens the steels, and also lowers their ductility to an undesirable degree. Additional treatment of the silicon-killed steels with a small amount of boron as contemplated by the present invention compensates for these undesirable effects of silicon and enables the production of silicon-killed steels of excellent deep drawing characteristics.

While specific examples have been given in the foregoing specification, these examples are given merely to illustrate the principles of the invention and the invention is not limited to or by such examples.

We claim:

1. Deep drawing silicon-killed steel containing between 0.01% and 0.1% carbon, 0.10% to 1% manganese, 0.05% to 0.50% silicon, 0.0005% to 0.05% boron, remainder iron and incidental impurities; and said steel being substantially free from deoxidizing elements, and deoxidation products thereof, other than said manganese, silicon, and boron.
2. Deep drawing silicon-killed steel containing 0.04% to 0.07% carbon, 0.10% to 0.50% manganese, 0.10% to 0.30% silicon, 0.001% to 0.02% boron, remainder iron and incidental impurities, said boron addition serving to counteract the hardness imparted by the silicon addition; and said steel being substantially free from deoxidizing elements, and deoxidation products

40

5

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

and composed of a silicon-killed steel containing 0.04% to 0.07% carbon, 0.10% to 0.50% manganese, 0.10% to 0.30% silicon, 0.001% to 0.02% boron, remainder iron and incidental impurities, said steel being characterized in that it has enhanced deep drawing characteristics over a silicon-killed steel of similar composition containing no boron; and said steel being substantially free from deoxidizing elements, and deoxidation products thereof, other than said manganese, silicon, and boron.

5. A method of preparing deep drawing steel comprising preparing a melt of low carbon steel containing carbon in an amount less than 0.10%

of said melt, treating said melt with silicon and boron in an amount sufficient to deoxidize and kill the same and to introduce between 0.0005% and 0.05% boron but insufficient to leave a residual silicon content greater than 0.30% of said melt.

10 6. A method of preparing deep drawing steel as claimed in claim 5 wherein the silicon and boron are added in the form of an iron-manganese-silicon-boron alloy comprising 20% to 60% manganese, 60% to 20% silicon, 1% to 15% boron, remainder iron and other incidental impurities.

WALTER CRAFTS.  
CECIL G. CHADWICK.